

## UNITED STATES PATENT OFFICE

2,164,930

## PROCESS FOR REDUCING VAT DYESTUFFS

Herbert August Lubs, Wilmington, Del., assignor  
to E. I. du Pont de Nemours & Company, Wil-  
mington, Del., a corporation of Delaware

No Drawing. Application November 10, 1937,  
Serial No. 173,848

8 Claims. (Cl. 8—34)

This invention relates to a novel process for reducing vat dyestuffs, and may be applied to the arts of dyeing, printing, discharging, preserving, stripping or other operations involving the coloring of textile fiber with vat dyestuffs or the removal of such color from the fiber. More particularly, this invention relates to a new assistant for the dyeing of textile fibers particularly those of vegetable origin such as cotton, 5 linen and regenerated cellulose with vat dyes by a process in which in some cases a leuco compound of a vat dye is formed prior to the introduction of the fiber to be dyed and in other cases a leuco compound is formed in the presence 10 of the fiber to be dyed, as, for example, by a printing process or a pad-jig dyeing process. It relates also to processes for the removal of the color in toto from dyed textile fibers, commonly known as stripping and to the production of 15 white or colored pattern effects on textile materials by the process commonly known as colored or white discharging or reserve printing. This invention further comprises novel 20 compositions of matter which are contemplated 25 for use in my improved processes above referred to, and which facilitate the carrying out of my invention.

It is well known that vat dyes are solid substances, insoluble in water, and that in order to 30 render them useful for the dyeing of textile fibers it is necessary to reduce them to the water soluble or so-called "leuco" form so that they may be taken up by the fiber. The fiber, im- 35 pregnated with the reduced water soluble dyestuff, is then subjected to an oxidizing or "fixing" treatment whereby the vat dyestuff is again converted to the insoluble form (the "Keto" form).

Hitherto, the hydrosulfites and the aldehyde 40 condensation products of hydrosulfites have been used almost exclusively for the conversion of vat dyes to their water soluble forms as well as for the reductive removal of the color from dyed fabrics. The processes of U. S. P. 746,784 of December 15, 1903, of U. S. P. 744,501 of November 45 17, 1903, and of U. S. P. 808,443 of December 26, 1905, are practically identical with the current processes for dyeing, discharging and printing, respectively, with vat dyestuffs. These 50 patients and accumulated experience show that two different agents, sodium hydrosulfite and form-

aldehyde sulfoxylate, are required for the various processes of dyeing, printing, and discharging. Because of its instability at elevated temperatures sodium hydrosulfite is unsatisfactory for use in the commonly practiced printing procedures. Because of its inactivity under the usual dyeing conditions, sodium formaldehyde sulfoxylate is unsatisfactory for use except for printing.

The present invention is based on the discovery that the product resulting from the oxidation of thiourea in neutral solution with hydrogen peroxide is eminently useful for the various processes for the application of vat dyestuffs to textile fibers and to the stripping of 10 color by reductive processes from dyed fabric. The oxidation product, known as thiourea-dioxide, imino-amino methane sulfonic acid, or formamidine-sulfonic acid, was first made and 15 described by Barnett (J. Chem. Soc. 97, 63-65; 1910). It was later observed that an ammoniacal solution of this compound is a powerful reducing agent for certain inorganic substances. (Boeseken, Koninklijke Akad. Wetenschappen, 20 Amsterdam, 39, 717-721; Receuil des Travaux 25 Chimique des Pays Bas, 55, 1040-1045; 1936). But that it had the power to reduce organic substances, and in particular to reduce vat dyestuffs to the leuco stage without destroying the dyestuff, has apparently not been known to date.

It must be observed here that the reduction of vat dyestuffs is a delicate operation, since there are many reduction stages possible, but only a particular one is desired. For instance, 30 in the case of anthraquinone itself, the reduction thereof may produce various successive stages of reduction known as hydro-anthraquinone, leuca-anthraquinone, hydroxy-anthrone, 35 hydroxy-anthranoil, anthrone, anthranol, etc., all the way down to anthracene or even dihydro-anthracene. Some of these compounds are tautomers, while two of the other members mentioned in the above group are probably identical respectively with "leuco-anthraquinone" and 40 "hydro-anthraquinone". The tautomers are nevertheless producible by different methods, and the "hydro" form cannot be used where the 45 "leuco" form is required.

It is known that certain reducing agents will 50 lead preferentially to one or another of the above

reduction stages, while others will give a mixture of several reduction stages simultaneously. (See Houben, *Das Anthracen und die Anthrachinone*, pages 143-147.) Under certain conditions the reduction may lead further to compounds of the dianthryl and dianthranol types. (*Ibid*, pages 172-183.)

It is clear from the above, that to be a useful reducing agent for vat dyestuffs, a given reagent must not only be capable of carrying the reduction to the desired degree, but must also be selective; that is, it must not produce the other reduction products to any appreciable extent. Considering further other prerequisites of a physical or economic nature, for instance stability at various temperatures of practical operation, solubility in caustic, or cost, it becomes clear why commercial practice has hitherto been confined practically to the single compound sodium hydrosulfite for dyeing and to the limited sulfoxylate group for printing.

I have now discovered that formamidine sulfonic acid has physical and chemical properties such as to adapt it ideally for the commercial reduction of vat dyestuffs. Moreover, I found that its stability over various ranges of temperature is so good that it may be applied with equal success to dyeing and printing; discharging, resisting and stripping. My invention accordingly consists of a process for the reduction of vat dyestuffs to their so-called "leuco"-stage, which comprises treating said dyestuffs with the reaction product of thiourea and hydrogen peroxide, in the presence of alkali, following in all other respects the details of procedure employed by the art in conjunction with the standard reducing agents, namely sodium hydrosulfite, and sodium-formaldehyde-sulfoxylate or other compounds of this class. My invention further comprises novel processes for reducing vat dyestuffs with the above mentioned reaction product, under conditions to which the hitherto standard reducing agents have not been applicable.

My novel process has the advantage over the processes of the art in being more versatile; in other words, the same reducing agent is applied to all processes wherein the reduction of a vat dye becomes necessary, including the processes of vat dyeing, pigment padding, printing, resisting, discharging and stripping. Another advantage lies in the fact that by virtue of the higher reducing value of formamidine-sulfonic acid not more than  $\frac{1}{2}$  to  $\frac{2}{3}$  of it by weight is used as compared with hydrosulfite or sulfoxylate. Furthermore, its stability in neutral and acid solutions permits of the development of novel application methods hitherto impossible with the known reducing agents. For instance, when my novel reducing agent is employed in printing, the subsequent step of ageing with steam may be omitted altogether or may be delayed for a considerable time, even several days, after the application of the printing paste, whereas in the sulfoxylate process immediate ageing is necessary at the penalty of producing inferior prints. My novel reducing agent also possesses greater stability in alkaline solution than sodium hydrosulfite. This fact enables me to produce vats of greater stability.

The versatility of my novel process is illustrated by the following examples which show the application of formamidine-sulfonic acid as a reducing agent under most varied conditions to

various processes of coloring fabric and removing color therefrom.

It is generally known that one method for the application of vat dyes to the dyeing of textile fibers is to apply the dye in unreduced form to the material, convert the dye to the water-soluble, reduced form on the fiber, in which form it is taken up by the fiber, and subsequently to fix the dye, as for example by oxidation, and finish the material by the customary processes. If the material is to be dyed a solid color, the "pad-jig" or "pigment-padding" process may be employed. If the color is to be applied locally in the form of a pattern or design, a "printing" process is utilized.

The following examples are given to illustrate the practical mode of operation in the various applied arts without, however, limiting my invention to any details of procedure. Parts mentioned are by weight.

#### I. DYEING BY THE PIGMENT PADDING METHOD 20

##### Example 1

Cotton cloth, preferably in open form, is passed through a liquor heated to 120 to 140° F. containing in suspension 16 ounces per gallon of a double paste of the dye described in Example 5 of U. S. Patent No. 1,705,023, and containing further formamidine sulfonic acid in the proportion of 4 ounces per gallon; it is then passed between squeeze rolls to remove surplus liquor and dried, preferably in open form, by any convenient means and temperature, but preferably not above 200° F. The fabric is next immersed for 3 minutes in a bath heated to 180 to 190° F. and containing 1 ounce per gallon of caustic soda. It is then passed between squeeze rolls and then treated for 1 to 3 minutes in a bath heated to 120 to 140° F. containing  $\frac{1}{4}$  to 1 ounce per gallon sodium or potassium di-chromate and  $\frac{1}{2}$  to 2 ounces per gallon of acetic acid (56%), then rinsed thoroughly by passage through water and then treated for 3 minutes in a bath heated to 200 to 212° F. containing  $\frac{1}{4}$  to 1 ounce per gallon soap. It is then rinsed and dried. The result is a uniformly dyed cloth of greenish yellow shade, possessing exceptional fastness properties.

The above example illustrates a novel application method made possible by the use of the new reducing agent. Neither sodium hydrosulfite nor a formaldehyde sulfoxylate derivative is applicable under these conditions.

##### Example 2

Cotton cloth, preferably in open form, is passed through a liquor heated to 120 to 140° F. containing in suspension 16 ounces per gallon of a double paste of the dye made according to Example 1 of U. S. Patent No. 1,761,624, and in solution 4 ounces per gallon formamidine sulfonic acid. It is then passed between squeeze rolls and dried, preferably in open form, by any convenient means and temperature but preferably not above 200° F. The fabric is next immersed for 3 minutes in a bath heated to 180 to 190° F. and containing 2 to 4 ounces per gallon caustic soda; then passed between squeeze rolls and then treated for 1 to 3 minutes in a bath heated to 120 to 140° F. containing  $\frac{1}{4}$  to 1 ounce per gallon sodium or potassium di-chromate and  $\frac{1}{2}$  to 2 ounces per gallon of acetic acid (56%), then rinsed thoroughly by passage through water and then treated for 3 minutes in a bath heated to 200 to 212° F. containing  $\frac{1}{4}$  to 1 ounce per gallon soap. It is then rinsed and dried. The result-

ing cloth is dyed uniformly in a navy blue shade of excellent fastness qualities.

*Example 3*

5 The procedure is the same as in Example 2, but the dyestuff employed is a double paste or powder of dimethoxy-dibenzanthrone Color Index No. 1101. The result is a brilliant green, uniform dyeing of excellent fastness qualities.

10 *Example 4*

Cotton cloth, preferably in open form, is passed through a liquor heated to 120 to 140° F. containing in suspension 4 ounces per gallon of a 13% paste of 4,4'-dimethyl-6,6'-dichlor thioindigo and

15 in solution 2 to 4 ounces formamidine sulfonic acid, then passed through squeeze rolls, dried, then immersed for 3 minutes in a bath heated to 180 to 190° F. and containing ½ to 1 ounce per gallon caustic soda; then passed between squeeze rolls and then treated for 1 to 3 minutes in a bath heated to 120 to 140° F. containing ¼ to 1 ounce per gallon sodium or potassium di-chromate and ½ to 2 ounces per gallon of acetic acid (56%), then rinsed thoroughly by passage through water 20 and then treated for 3 minutes in a bath heated to 200 to 212° F. containing ¼ to 1 ounce per gallon soap. It is then rinsed and dried.

25 *Example 5*

30 Cotton cloth is treated exactly as described in Examples 1 to 4 inclusive and with the dyes therein described, except that after passage through the liquor containing the dye and the formamidine sulfonic acid it is treated in the caustic soda solution without previous drying.

35 *Example 6*

40 Cotton cloth, preferably in open form, is passed through a liquor heated to 120 to 140° F. containing in suspension 16 ounces per gallon of the dyes mentioned in Examples 1 to 4 inclusive, and in solution 4 ounces per gallon formamidine sulfonic acid, passed through squeeze rolls, dried and then passed through 15 to 30% solution of caustic soda heated to 80 to 140° F. It is then treated 45 in an ager or chamber containing moist steam and heated to a temperature of 160 to 220° F. for 3 to 30 minutes. It is then oxidized and finished as described in Examples 1 to 4.

50 *Example 7*

55 Cotton cloth, preferably in open form, is treated exactly as described in Example 6 and with the dyes therein mentioned, except that after passage through the liquor containing the dye and the formamidine sulfonic acid, it is passed through the caustic soda bath, and eventually through the ager, without previous drying.

60 The above examples, 1 to 7 inclusive, relate to the dyeing of cotton cloth. It is to be understood that the process is applicable to linen, and the synthetic fibers and combinations of these in woven, knitted and other manufactured or coherent structures.

65 **II. DYEING FROM THE REDUCED VAT**

The use of formamidine sulfonic acid for the application of vat dyes in reduced form is shown by the following examples:

70 *Example 8*

4 lbs. of a double paste of 1,5-dibenzoylaminanthraquinone (Color Index 1132) are reduced in 10 gallons of water with 3 lbs. of caustic soda and 2 to 3 lbs. of formamidine sulfonic acid for

20 minutes at a temperature of 120° F. In the interval, to 80 gallons of cold water is added 4 ounces of caustic soda and 4 ounces of formamidine sulfonic acid. The reduced dye is added to this latter and 50 lbs. of cotton cloth or yarn are 5 entered into it and treated for from 30 to 60 minutes. The cotton is then removed, and after removing excess moisture by any convenient means, it is oxidized at 120 to 140° F. in a bath containing ¼ to 1 ounce per gallon of sodium or 10 potassium di-chromate and ½ to 2 ounces per gallon acetic acid (56%), then thoroughly rinsed with water and finished by treatment in a boiling soap solution.

15 *Example 9*

10 lbs. of a single paste of 6,6'-diethoxy-2,2'-bis-thionaphthen-indigo (Color Index 1217) are reduced in 100 gallons of water containing 4 to 5 lbs. caustic soda and 2 to 3 lbs. of formamidine sulfonic acid for 20 minutes at 140° F. 50 lbs. of cotton cloth or skeins is treated in this for from 30 to 60 minutes and then oxidized and finished as described in Example 8.

25 *Example 10*

30 30 lbs. of a double paste of nitrated dibenzanthrone (Color Index 1102) is reduced in 50 gallons of water containing 10 lbs. caustic soda and 3 to 35 6 lbs. of formamidine sulfonic acid for 20 minutes at 140° F. In the interval, 1 lb. of caustic soda and 4 ounces of formamidine sulfonic acid are dissolved in 50 gallons of water. The reduced dye is added to this and 50 lbs. of cotton cloth or skeins are entered and stirred for 15 to 30 minutes. To assist penetration of the dye into the fiber and a more complete exhaustion of the dye bath the temperature is then raised to 160 to 200° F. and treatment continued for 15 to 30 40 minutes longer. The cotton is removed, oxidized and finished as described in Example 8.

**III. DYEING UNDER VARIOUS SPECIAL CONDITIONS**

45 My novel process is also adapted for vat dyeing in a circulating liquor machine, for instance the Franklin or Chatanooga machine, as is illustrated by Examples 11 to 13 below.

50 When applying some of the vat dyes in machines as well as in open vessels it is customary to use as assistants, substances such as animal glue, sulfite waste liquor and others, to retard the rate at which the dyes are absorbed and thus aid their uniform absorption and penetration into the fibers. It is also well known that raising the temperature of the dye baths to between 180 and 200° F. toward the end of the operation, after all or the greatest quantity of the dyes has been absorbed, will aid their uniform distribution 55 through the material and their penetration into the fibers. This reduces the tendency of the dye on the material to rub off and stain other materials with which it may come into contact. It will also in many instances beneficially influence the resistance of the color to the destructive agencies to which the fibers are subjected during the manufacturing processes and in subsequent use.

60 Under many of these conditions sodium hydro-sulfite is inapplicable because of its insufficient stability at the higher temperatures. My novel process, however, using formamidine sulfonic acid 65 may be readily carried out under these special conditions.

**Example 11**

100 lbs. of loose cotton is placed in a circulating liquor type machine and wet out as is customary, by treating with boiling water containing small quantities of sodium carbonate or other wetting agents. In the interval 5 to 30 lbs. of the paste or powder types of any of the dyes known by the trade name of

- 10 Ponsol Yellow G (C. I. 1118)  
 Ponsol Golden Orange G (see Color Index Supplement p. 50)  
 Ponsol Violet RRD (C. I. 1104)  
 Ponsol Dark Blue DR (C. I. 1099)

15 are reduced in 20 to 50 gallons of water, containing 8 to 10 lbs. of caustic soda and 3 to 6 lbs. of formamidine sulfonic acid by stirring the ingredients together for 20 minutes at 140° F.

After the loose cotton is thoroughly and uniformly wetted, the liquor is drained, the machine is partly filled with water; this is heated to 80° F., and 4 to 8 ounces of caustic soda and 4 ounces formamidine sulfonic acid are added.

This liquor is circulated for 5 to 15 minutes, 25 the reduced dye is added, the liquor is circulated with reversal of its flow and the temperature is raised gradually within 45 minutes to 180 to 200° F. and there maintained for 15 to 30 minutes. This liquor is then drained, the stock is rinsed 30 with cold water, oxidized with 1 to 2% of its weight of sodium perborate and again well rinsed in cold water containing 5 to 15 lbs. of common salt (sodium chloride) or small quantities of other substances that aid manufacturing operations, 35 and then dried.

**Example 12**

The procedure is as described in the preceding example, except that the dyes used are those 40 known in the trade as Sulfanthrene Blues G and GR, (Color Index Supplement page 53), and their reduction is effected with 2 to 5 lbs. caustic soda and 1½ to 3 lbs. of formamidine sulfonic acid.

**Example 13**

100 lbs. of cotton or linen yarn in package form, or in loose form, is dyed in a circulating liquor type machine by first thoroughly wetting 50 with boiling water, with or without the aid of wetting and penetrating assistants. This liquor is then drained, the machine partly filled with water, this is heated to 140 to 160° F. and circulated for a short time, with or without the 55 addition of dispersing and penetrating assistants. 5 to 30 lbs. of the paste or specially prepared easily dispersible powders, known to the trade as the Grain or S types, of the dyes described in Example 11, are uniformly dispersed in 10 to 30 gallons of cold water, added to the machine and the liquor circulated for a short time. 8 to 10 lbs. of caustic soda in any convenient strength of 60 solution is added, circulation is continued for 15 to 30 minutes; 3 to 6 lbs. of formamidine sulfonic acid are added and circulation continued for another 15 minutes; the temperature is then raised to 180 to 200° F. and circulation continued for 15 to 30 minutes longer. Rinsing, oxidation and finishing follow by the means usually employed 70 for processes of this kind.

While formamidine sulfonic acid is extremely valuable because of its stability at elevated temperatures, it is also useful for the reduction and application of the vat dyes normally applied at 75 temperatures between 80 to 120° F.

**IV. DYING OF WOOL WITH INDIGO****Example 14**

Prepare a stock vat as follows:

|                           | Parts |   |
|---------------------------|-------|---|
| A 20% indigo paste        | 215.0 | 5 |
| Caustic soda              | 24.0  |   |
| Formamidine sulfonic acid | 25.0  |   |

make up to 1000 parts with water; reduce for 20 minutes at 130° F.

From the above stock vat a dye bath for wool may be prepared as follows:

|                           | Parts |    |
|---------------------------|-------|----|
| Stock vat                 | 35.0  |    |
| Ammonia (.880)            | 1.2   | 15 |
| Formamidine sulfonic acid | .75   |    |

Glue make up to 100 parts with water; dip 25 parts of wool for 10 minutes at 120° F.

Squeeze the material, allow to air-oxidize for 20 about 5 to 10 minutes and give a good rinsing, then dry. The dye bath may be used continuously by replenishing the indigo by additions of stock vat and formamidine sulfonic acid after each dip and ammonia and glue after 4 or 5 successive dips. The amounts to be added must be determined by experiment in each particular case.

**V. DYEING—IN GENERAL**

While specific quantities of the dyes are mentioned in the above examples, these quantities may be varied within wide limits depending upon the tintorial strength of the shade desired. The quantity of the formamidine-sulfonic acid required may also be varied accordingly, and, whereas in the examples cited the temperature and time for the application of the dye together with the formamidine-sulfonic acid as well as the temperature and time for subsequent reduction in the caustic soda solution is described, these also may be varied to advantage between room temperature, 70 to 80° F., and 212° F. and between 1 and 30 minutes, depending upon the material and character of the individual dyes. Whereas in the examples cited oxidation is effected with chrome and acetic acid it can be equally satisfactorily accomplished by exposing the material in air or by treatments for suitable periods of time and temperatures in baths containing .05 to .25 ounce per gallon sodium perborate or hydrogen peroxide or solutions of sodium hypochlorite containing .01 to .05% available chlorine.

When sodium perborate or hydrogen peroxide is used as the oxidation medium the finishing operation by soaping at the boil may be effected by adding the required quantity of soap to the oxidation baths and raising the temperature to the boil.

The necessity and convenience of variation in the procedure for the application of the vat dyes is well known and recognized in the art of dyeing and is dependent upon the type of apparatus used, form in which the material is colored and other variables in local conditions.

Rayon, linen, silk and wool, the latter with the aid of protective colloids, alone or in combination, may be dyed with the dyes and under the conditions described in the above examples.

In addition to the dyes specifically described in the above examples, many others have been satisfactorily applied under the conditions described and produced commercially satisfactory results in relation to penetration of the cloth, uniformity of its appearance and resistance to

the natural destructive agencies which this class of dyes resists when applied under the conditions at present in practical use. The dyes thus tested include among others:

- 5 Ponsol Blue BCS (Color Index 1114)  
 Ponsol Blue GD (Color Index 1113)  
 Caledon Brown R (Color Index 1151)  
 Caledon Brown G (Color Index 1152)  
 10 Caledon Red FF (Color Index Supplement p. 30)  
 Caledon Olive (Color Index Supplement p. 30)  
 Caledon Golden  
 Orange G (Color Index Supplement p. 30)

#### VI. PRINTING OF FABRIC

- 15 Formamidine sulfonic acid can be used in the printing of vat colors either by incorporating the formamidine sulfonic acid in the usual printing composition of color, alkali, thickener and hydro-  
 20 tropic and hygroscopic agent, or by including the formamidine sulfonic acid in with the dye as a powder or as a paste, in which case no further addition of formamidine sulfonic acid or other reducing agent need be made to the printing paste.  
 25 In addition to direct printing, formamidine sulfonic acid can be satisfactorily used for the production of white or colored discharges and in resist printing.  
 30 The unusual properties of formamidine sulfonic acid which distinguish it from the usual reducing agent used in printing, namely sodium sulfoxylate formaldehyde, are its exceptionally strong and rapid reducing action in the presence  
 35 of alkali which enables satisfactory prints to be obtained with much less of formamidine sulfonic acid than of sodium sulfoxylate formaldehyde; it also allows satisfactory prints to be made with  
 40 a shorter than normal aging period (say 3 to 6 minutes against 5 to 10 minutes); and since reducing fumes, such as formaldehyde or sulfur dioxide, are not given off in the aging process, it permits the printing of azoic colors in the same  
 45 pattern along with vat colors.

#### Example 15

A printing paste prepared as follows:

|                                                                  | Parts  |
|------------------------------------------------------------------|--------|
| 50 Dimethoxy dibenzanthrone, double paste,<br>(Color Index 1101) | = 20.0 |
| Formamidine sulfonic acid                                        | = 5.0  |
| Sodium hydroxide (35%)                                           | = 5.0  |
| 55 Potassium carbonate                                           | = 10.0 |
| Glycerin                                                         | = 5.0  |
| Starch—British gum thickener                                     | = 55.0 |
|                                                                  | 100.0  |

- 60 This printing paste may be applied to cotton or rayon fabric by such means as the usual roller printing machine, by engraved blocks, by stencil, or by screen. After the dye paste has been applied to the fabric the latter is dried, preferably in a current of warm air, and "aged" for 3 to 6 minutes in a vat color aging device such as the Mather-Platt ager or in a "Schnelldamfer". It is then oxidized for 45 seconds in a bath containing  $\frac{1}{2}\%$  acetic acid plus  $\frac{1}{2}\%$  sodium bichromate heated to 120° F., then rinsed free of acid, soaked for 5 minutes in  $\frac{1}{2}\%$  soap solution at 180° F., rinsed and dried. A green print of exceptional strength, levelness and brightness is obtained.

#### Example 16

A printing paste prepared as follows:

|                                       | Parts  | 5  |
|---------------------------------------|--------|----|
| Tetra bromo indigo paste (C. I. 1184) | = 20.0 |    |
| Formamidine sulfonic acid             | = 5.0  |    |
| Sodium hydroxide (35%)                | = 5.0  |    |
| Potassium carbonate                   | = 10.0 |    |
| Glycerin                              | = 5.0  | 10 |
| Starch—British gum thickener          | = 55.0 |    |
|                                       | 100.0  |    |

This printing paste is applied to cotton or rayon fabric and subjected to the usual operations of drying, aging, oxidation and soaping as in Example 15. A blue print of exceptional brightness, levelness and strength is obtained.

#### Example 17

A printing paste prepared as follows:

|                                       | Parts  | 25 |
|---------------------------------------|--------|----|
| Ciba brown G (C. I. Supplement p. 34) | = 20.0 |    |
| Formamidine sulfonic acid             | = 5.0  |    |
| Sodium hydroxide (35%)                | = 5.0  |    |
| Potassium carbonate                   | = 5.0  |    |
| Sodium dibenzyl aniline sulfonic acid | = 2.0  |    |
| Starch—British gum thickener          | = 58.0 | 30 |
|                                       | 100.0  |    |

This paste is applied to the fabric and subjected to the same developing and finishing operations as in Example 15. A bright, strong and lever brown print is obtained.

#### Example 18

A vat color printing paste is prepared by mixing and milling as in a paint mill, 50 parts by weight of dimethoxy dibenzanthrone, double paste (C. I. 1101), 25 parts by weight of formamidine sulfonic acid and 25 parts by weight of water. 20.0 parts of this paste are then incorporated with

|                              | Parts | 40 |
|------------------------------|-------|----|
| Potassium hydroxide (50%)    | 5.0   |    |
| Potassium carbonate          | 10.0  |    |
| Glycerin                     | 5.0   | 45 |
| Starch—British gum thickener | 60.0  |    |
|                              | 100.0 |    |

This paste is applied to the fabric and subjected to the same developing and finishing operations as in Example 15. A bright, level green print is obtained.

#### VII. JOINT PRINTING WITH VAT AND AZOIC COLORS

60

#### Example 19

A vat color printing paste may be prepared and printed in the same pattern with an azoic color as follows:

65

#### VAT COLOR

|                                     | Parts | 75 |
|-------------------------------------|-------|----|
| Anthraflavone GC paste (C. I. 1095) | 20.0  |    |
| Formamidine sulfonic acid           | 5.0   |    |
| Sodium hydroxide (35%)              | 8.0   | 70 |
| Potassium carbonate                 | 15.0  |    |
| Glycerin                            | 5.0   |    |
| Starch—British gum thickener        | 47.0  |    |
|                                     | 100.0 |    |

## AZOIC COLOR

|                                           | Parts |
|-------------------------------------------|-------|
| Red azoic composition as described in Ex. |       |
| 21 of U. S. P. 1,882,561                  | 4.0   |
| 5 Sodium hydroxide (35%)                  | 1.5   |
| Water                                     | 24.5  |
| Starch—tragacanth thickener               | 70.0  |
|                                           | 100.0 |

- 10 The vat and azoic colors may be applied to cotton fabric by one or another of the customary printing devices in a pattern on which the two classes of colors are adjacent. The fabric is then dried, aged in a vat color ager, such as the 15 Mather-Platt type, for 5 minutes, then aged in an acid fume ager for 3 minutes; it is then oxidized for 5 minutes in a bath of 1% sodium perborate plus 1% acetic acid at 120° F. then rinsed and soaped in the usual manner. A bright yellow 20 and red design is obtained in which there is no dulling or discharge of the azoic color where it touches the vat color.

## Example 20

- 25 A vat color may be printed in conjunction with an azoic color by a novel modification of the familiar Colloresin printing process, which comprises the addition of the reducing agent to the 30 vat color printing paste. This procedure has heretofore been impossible.

## VAT COLOR PRINTING PASTE

|                                               | Parts |
|-----------------------------------------------|-------|
| Dimethoxy dibenzanthrone, single paste (C. I. |       |
| 35 1101)                                      | 20    |
| Formamidine sulfonic acid                     | 5     |
| Methyl cellulose (5%)                         | 75    |

## AZOIC COLOR

|                                           | Parts |
|-------------------------------------------|-------|
| Red azoic composition as set forth in Ex. |       |
| 20 of U. S. P. 1,882,561                  | 4.0   |
| Ethylene glycol-mono-ethyl-ether          | 4.0   |
| Sodium hydroxide (35%)                    | 1.5   |
| 45 Water                                  | 20.5  |
| Starch—tragacanth thickener               | 70.0  |
|                                           | 100.0 |

- 50 The vat and azoic colors may be applied by one of the customary printing devices to a pattern on which the two classes of colors are adjacent, dried, aged for 3 minutes in an acid fume ager, air dried, slop-padded in a solution containing 20% potassium carbonate and 5% glycerin, dried and aged 4 minutes in a Mather-Platt ager, oxidized for 45 seconds in a bath containing 1/2% acetic acid plus 1/2% sodium bichromate at 120° F., rinsed and soaped in the usual manner. A bright, level red and green pattern in which 55 there is no dulling or bleeding of the green vat color or dulling or discharge of the red azoic color is obtained.

- 60 In a similar manner other combinations of vat dyes and azoic colors may be printed in the same pattern or textile fabric. The azoic colors for this purpose are preferably selected from the class which may be broadly defined as a coloring composition comprising a stabilized diazonium compound, preferably one stabilized by the aid of the salt of a secondary amine, in admixture with an azo-coupling component, preferably one of the type which develop into a water-insoluble dye, for instance one of the arylides of 2,3-hydroxynaphthoic acid.

The development of the print on the fiber may, as illustrated by the above examples, follow either one of two procedures: The fabric may be treated first in a vat-dye ager and then in an acid fume ager, or the procedure may be reversed. 5 This freedom of procedure is a special, advantageous feature of my novel process of reduction and does not exist where the hitherto standard reducing agents are employed.

## VIII. DISCHARGING

## Example 21

Cotton goods dyed with tetra bromo indigo paste (C. I. 1184) printed in the usual manner 15 with a past of the following compositions:

|                                         | Parts |
|-----------------------------------------|-------|
| Zinc oxide 50% paste                    | 200   |
| Anthraquinone 30% paste                 | 50    |
| Formamidine-sulfonic acid               | 150   |
| Dimethyl-benzyl-phenylammonium chloride | 100   |
| Caustic soda 76° Tw                     | 100   |
| British gum thickening                  | 400   |
|                                         | 35    |
| Total                                   | 1000  |

After printing, the goods are steamed, passed through silicate of soda, and then soaped in the usual manner, as described for instance on page 50 613, *The Principles and Practice of Textile Printing*, E. Knecht and J. B. Fothergill. (London, 1936.)

## Example 22

|                                                                 | Parts |
|-----------------------------------------------------------------|-------|
| 5,5'-dichloro-6,6'-dimethyl-2,2'-bisthiophenindigo (C. I. 1212) | 20.00 |
| Formamidine sulfonic acid                                       | 8.0   |
| Sodium hydroxide (35%)                                          | 8.0   |
| Potassium carbonate                                             | 10.0  |
| Glycerin                                                        | 5.0   |
| Starch—British gum thickener                                    | 49.0  |
|                                                                 | 45    |
| Total                                                           | 100.0 |

The above printing paste when applied on a fabric dyed with a dischargeable azoic color by one of the usual printing methods followed by the developing and finishing operations as in Example 15 yields a sharply defined reddish-violet discharge design on the dyed ground.

## IX. RESIST PRINTING ("RESERVE PRINTING")

## Example 23

The vat color printing paste as formulated in Example 15 may be locally resisted by preprinting the fabric with a resist design of the following composition:

|                                          | Parts |
|------------------------------------------|-------|
| British gum (40%)                        | 60    |
| Dimethyl-benzyl-phenyl-ammonium chloride | 10    |
| Potassium carbonate                      | 12    |
| Zinc oxide-glycerin mixture              | 10    |
| Formamidine-sulfonic acid                | 8     |
|                                          | 65    |
|                                          | 70    |
| Total                                    | 100   |

A fabric printed with the above resist paste is overprinted without drying with the vat color printing paste as given in Example 15 and developed and finished by the customary operations as in Example 15. A bright white "resist" design stands out against a brilliant green setting where the "resist" paste has been applied.

*Example 24*

The procedure is the same as in Example 23, but the resist paste is prepared from the following ingredients:

|                                 | Parts |
|---------------------------------|-------|
| m-Nitrobenzene-sodium-sulfonate | 15    |
| Water                           | 25    |
| Gum thickener                   | 60    |
|                                 | 100   |

10 A bright white resist design is obtained.

**X. STRIPPING***Example 25*

50 parts of cotton, linen, rayon or mixtures of these, in the form of cloth or yarn, previously colored with vat dyes are treated in 1000 parts of water containing

|                                                                                                     | Parts     |
|-----------------------------------------------------------------------------------------------------|-----------|
| Cetyl-trimethyl-ammonium bromide, with or without oleic acid (see U. S. P. 2,003,928 and 2,019,124) | 0.25 to 5 |
| 25 Caustic soda                                                                                     | 1.5 to 3  |
| Formamidine-sulfonic acid                                                                           | 1. to 5   |

The above materials may be added to the bath either before or after entry of the textile material. In either event, the bath is heated to a temperature of 120 to 140° F. at the beginning of the treatment, and is then gradually raised in temperature to at least 200° F., and preferably 212° F., the treatment being continued with suitable agitation of the material for from 30 to 60 minutes. The source of heat is then removed, and cold water is run in, permitting the excess to flow away through any suitable arrangement, until all of the original liquor has been displaced. This water is then drained and 1000 parts of a ½° Tw. solution of sodium hypochlorite is added, and the material is treated in it at a temperature between 65 and 80° F. for 20 to 30 minutes. This is followed by the usual rinsing in cold water, or treatment in cold solutions of sodium thiosulfate or of other suitable substances to remove the residual hypo-chlorite. This treatment will remove some or all of the color, depending upon the dye or dyes and their quantity that the material originally contained.

50 Among the vat dyes that are completely or nearly completely removed by this treatment are

|                                                       |  |
|-------------------------------------------------------|--|
| Anthraflavone GC (C. I. 1095)                         |  |
| Caledon Brown R (C. I. 1151)                          |  |
| 55 Po'sol Blue GD (C. I. 1113)                        |  |
| Caledon Olive (see C. I. Supplement page 30)          |  |
| 6,6'-diethoxy-2,2-bisthionaphthen-indigo (C. I. 1217) |  |

**XI. DYEING WITH SULFUR COLORS***Example 26*

Paste 5 parts sulphur Black R (C. I. 978)  
50 parts water, and

|                                                                                                                                            |  |
|--------------------------------------------------------------------------------------------------------------------------------------------|--|
| 65 add 3.5 parts formamidine-sulfonic acid and 2.5 parts sodium hydroxide                                                                  |  |
| Add 350.0 parts of water, heat to 180° F. Enter the cotton goods to be dyed and hold at this temperature for 15 minutes                    |  |
| 70 Then add 30.0 parts of salt and continue the dyeing for 45 minutes longer.                                                              |  |
| Remove the dyed goods and finish by rinsing, oxidizing and drying in the usual manner. There is thus produced textile material dyed a fast |  |
| 75 black shade.                                                                                                                            |  |

*Example 27*

The procedure is the same as in Example 26 above, except that the dye prepared as in Example 1 of U. S. P. 1,944,250 is used in lieu of the color therein mentioned. There is thus obtained textile material dyed a blue shade of unusual fastness.

**XII. DYEING BY PREPARING REDUCING AGENT IN SITU**

10 It is a remarkable feature of my novel process that the reducing agent may be prepared in situ in the process of dyeing. For instance, one may proceed as follows:

*Example 28*

15 2 parts of thiourea are dissolved in 100 parts of water, and to this are added 30 parts of 3% hydrogen peroxide preferably keeping the temperature under 80° F.

To this solution there is then added 1 part of 20 13% paste of 4,4'-dimethyl-6,6'-dichlor-thiourido. Then there are added 2.5 parts of sodium hydroxide. The suspension thus formed is then heated at 180° F. until the reduction of the vat dyestuff is complete. The goods to be dyed are 25 then immersed in this solution, removed after 1 hour, and finished in the customary manner, including the steps of oxidation and soaping. The dyings thus obtained are as good as when the ordinary sodium hydrosulfite bath is employed.

*Example 29*

30 The procedure is the same as in Example 28, except that Anthraflavone GC is employed as 35 color. The results are very good.

In a similar manner tetrabromo indigo dyestuff paste or other vat dyestuffs may be dyed upon cotton or rayon goods, with slight variations, in some cases, of the temperature, caustic 40 concentration and dyeing time, to suit the best conditions for any particular dyestuff, as is well understood by those skilled in the art. If desired the vat dye may be mixed with the thiourea, or with the aqueous solution thereof, prior 45 to the treatment of the latter with the hydrogen peroxide.

**XIII. DYESTUFF COMPOSITIONS**

50 By virtue of the general stability of my preferred reducing agent in this invention, it is possible to compound the same with the dyestuff, either in powder form or in paste form, and to market the resulting composition as a 55 vat dye preparation which is adapted for direct use requiring no additional reagents for its solution except alkali. These dyeing preparations may contain further dyeing or printing assistants, for instance wetting agents, dispersing agents, etc., and may be prepared specially for 60 use in dyeing or for printing, or for both.

The following examples illustrate typical compositions in accordance with this particular feature of my invention.

*Example 30*

|                                                             | Parts |
|-------------------------------------------------------------|-------|
| Dimethoxy dibenzanthrone                                    | 21    |
| Cane sugar                                                  | 63    |
| Lauryl-sodium-sulfate                                       | 4     |
| Dextrin                                                     | 70    |
| Formaldehyde-naphthalene-sulfonic acid condensation product | 11    |
|                                                             | 1     |
| Total                                                       | 100   |
|                                                             | 75    |

100 parts of the above composition are mixed with 100 parts of formamidine-sulfinic acid and ground together until very fine.

5 This composition of material can be used for the production of brilliant green shades by dyeing and printing methods without further addition of reducing agent.

*Example 31*

10 50 parts of an aqueous double paste of tetrabromoindigo are mixed with 50 parts of formamidine-sulfinic acid and milled together until thoroughly uniform.

15 The resulting composition is satisfactory for use in the various processes of printing and dyeing, without further addition of any reducing agent.

*Example 32*

20 100 parts of tetrabromoindigo double paste are mixed with 60 parts of a polyhydric alcohol, such as ethylene glycol, and the whole is evaporated to a weight of 80 parts. There is then added 20 parts of formamidine-sulfinic-acid and the mass is intimately mixed by means of a suitable 25 grinder.

25 The assistant paste so produced is very satisfactory for use in the printing of textile fibers without further addition of reducing agent. Instead of the ethylene glycol there may be used 30 diethylene glycol, glycerine or a mixture of these materials with liquids such as the ethanolamines.

35 It will be understood that the above examples are merely illustrative, and that the details of my process are susceptible of wide variation and modification within the skill of those engaged in this art.

40 Thus, the alkalinity of the dyeing bath, printing paste, discharge paste or stripping bath, as the case may be, is generally to be selected in accordance with the practice of the art in regard to the particular dye employed when using hydrosulfites or sulfoxylates. It is well known that the alkaline concentration required for best results varies with the nature of the dye employed. 45 Some dyestuffs will not dissolve completely when reduced unless a strongly alkaline bath is employed. Dyestuffs of the indanthrene group, for instance, require such a strongly alkaline bath as to prohibit the application of the process to wool 50 fibers (Houben, *ibid*, page 31). Indigo on the other hand is very easily reducible and can be treated in a mildly alkaline bath, for instance an ammoniacal bath.

55 It will be clear from the foregoing, that the nature of the alkali employed, that is whether sodium-, potassium- or ammonium-hydroxide may likewise vary with the individuality of the dye employed, and will generally conform to the usual practice with such dye when hydrosulfite or sulfoxylate reducing agents are employed.

60 The nature of the operation, of course, is also determinative of the nature and strength of the alkali required. Thus, in ordinary pigment padding, a bath containing less than 1% of NaOH is often satisfactory. (Cf. Example 1, above.) Where, however, the pigment padding method is employed in conjunction with a steaming operation, a concentrated bath containing as high as 70 15 to 30% by weight of caustic soda may be employed. (Cf. Example 6.) Likewise, in printing, the alkali employed is generally in the form of a carbonate, for instance potassium or sodium carbonate. Sometimes, this may be used in conjunction with sodium or potassium hydroxide. 75

In all such details, the general rule which I recommend with my invention, is to follow the preferred practice of the art as if the particular operation concerned were carried out with the hitherto customary reducing agents (i. e. sodium hydrosulfite or the various sulfoxylates). 5

10 In other details, for instance temperatures, ingredients of the pastes, use of assistants, retarding agents, oxidizing agents, ageing procedures, etc., the process of my invention may follow the general practice of the art, as though the reducing agent were one of the standards heretofore in use.

15 My invention is applicable also to the reduction of sulfur colors, as well as to the reduction of indigo, indigoid colors and vat colors manufactured by a thionation process. Thioindigoid 20 colors and vat colors of the anthraquinone series have already been mentioned above. Accordingly, in the claims below, the term "vat dyestuff" shall be construed as a comprehensive term for all dyes which are water-insoluble and which are generally applicable to the fiber by a process involving first treatment of the dye with a reducing agent to produce an alkali-soluble reduction product of the dye (the so-called "leuco" form), and then re-oxidizing the dye on the fiber to convert it into its original water-insoluble form. The nature of the reducing agent hitherto employable or preferable for the reduction step, (whether a 25 hydrosulfite, a sulfoxylate, sodium sulfide, sugar or any other reducing agent) does not enter into the above definition of "vat dyestuff", and is not intended to limit the construction thereof in this application. 30

35 As regards the novel reducing agent employed by me in this invention, it will be understood that although I refer to it as formamidine-sulfinic acid, I do not intend thereby to limit my invention to any particular structure or any particular 40 form of this compound. A review of the literature concerning this compound shows that its structure is still somewhat in dispute. Some workers called this compound thiourea dioxide, implying a structure as in Formula I below. Other authorities refer to it as imino-amino-45 methane-sulfinic acid, implying a structure as in Formula II.



Formula I



Formula II

55 It is possible that both forms are correct, and that the compound spontaneously undergoes tautomeric rearrangement, depending on the medium it is in (whether acid or alkali) or on the temperature.

60 Furthermore, if the second formula be considered, it is conceivable that it forms a salt when in alkaline solution, for instance the sodium sulfinate when in sodium hydroxide solution. It is further conceivable that in acid solution it forms salts on the imino group, for instance a hydrochloride. 65

65 All the above are fine theoretical points which cannot readily be determined in practice.

70 Moreover, as shown above in Examples 28 and 29, instead of using the isolated formamidine-sulfinic acid, one may employ in my process materials which when brought together in aqueous solution form said compound in situ, for instance thiourea and hydrogen peroxide. It is to be understood therefore that in the claims below 75

when I speak of "formamidine-sulfinic acid", I am referring to the compound which is obtainable by oxidizing thiourea with hydrogen peroxide at a relatively low temperature, for instance around 5 0 to 10° C., and to any compound which is chemically identical therewith regardless of the mode of its synthesis, as well as to any tautomeric form thereof and to any salt thereof which behaves in alkaline solution in the same manner as an 10 alkaline solution of said compound, including further any combination of initial materials which when brought together in aqueous solution produce said compound in situ.

As regards the materials that may be dyed or 15 printed by my novel process, it will be understood that my invention is applicable to any of the materials heretofore employable with vat dyes. These may include cellulosic textile material, for instance cotton, rayon, cellulose acetate, or, in 20 certain instances, animal fiber such as wool. Then again the material may be in the form of textile fiber, for instance fabric or yarn, or it may be in the form of sheets, films or filaments, as for instance in Cellophane.

25 I claim:

1. In the process of converting a vat dyestuff into its leuco form, the step which comprises reducing the vat dyestuff by the aid of formamidine-sulfinic acid.
- 30 2. The process of reducing a vat dyestuff to its leuco form, which comprises treating the same with formamidine-sulfinic acid and alkali.
- 35 3. In the process of converting a vat dyestuff into its leuco form, the step which comprises reacting with alkali upon said vat dyestuff in the presence of formamidine-sulfinic acid at a temperature between 80 and 220° F.

4. The process of coloring textile material which comprises reacting with alkali and formamidine-sulfinic acid upon a vat dyestuff in contact with the textile material, and then subjecting the textile material to an oxidation treatment whereby to reconvert the vat dyestuff into 5 its water-insoluble form.

5. A process for dyeing cellulosic textile material which comprises padding the same with an aqueous suspension of a vat dye containing further formamidine-sulfinic acid, then treating the material in an alkaline aqueous bath whereby to effect reduction of the vat dye on the fiber to its leuco form, and subsequently oxidizing the 10 vat dye on the fiber whereby to reconvert the vat 15 dye into its water-insoluble form.

6. A process for dyeing textile material which comprises treating the same in a vat formed by reacting with alkali upon an aqueous mixture of a vat dye and formamidine-sulfinic acid, where- 20 by to impregnate the textile material with the reduced vat dye, and then further treating the textile material so impregnated with an oxidizing bath adapted to reconvert the reduced vat dye to its water-insoluble form.

7. A process of printing textile material, which comprises applying thereto locally a printing paste comprising a vat dye, formamidine-sulfinic acid, an alkali and a soluble gum, and then subjecting the printed material successively to steam 30 aging and to oxidation, whereby to develop the color upon the fiber.

8. A vat color preparation comprising, in intimate admixture, a vat dye and formamidine sulfinic acid.

35 HERBERT A. LUBS.